

Patented Sept. 2, 1924.

## UNITED STATES PATENT OFFICE.

PAUL DEUSSING, OF RUHLA, GERMANY, ASSIGNOR TO THE FIRM LÖWENSTEIN & CO.,  
OF FRANKFORT-ON-THE-MAIN, GERMANY.

## PROCESS FOR THE MANUFACTURE OF ARTIFICIAL MEERSCHAUM.

No Drawing.

Application filed June 1, 1921. Serial No. 474,225.

*To all whom it may concern:*

Be it known that I, PAUL DEUSSING, a citizen of the German Republic, residing at Ruhla, Germany, have invented certain new and useful Improvements in Processes for the Manufacture of Artificial Meerschaum, of which the following is a specification.

This invention relates to a process for the manufacture of artificial meerschaum which 10 on the one hand combines the excellent qualities of real meerschaum and on the other hand possesses certain advantages over the natural product. The objects made from the artificial meerschaum produced according to this invention are of the same colour as similar objects made from real meerschaum, have approximately the same weight and the same porosity as these. Pipe-bowls made from the artificial mass are 20 quite as nice in use as pipe-bowls made from real meerschaum as the artificial meerschaum manufactured according to this invention absorbs the tobacco juice quite as completely as this is done by real meerschaum, so 25 that in both cases the smoke reaching the mouth of the smoker is dry, of an agreeable and mild taste and absolutely free from biting and disagreeable effects.

The special advantages offered by the 30 artificial meerschaum compared with the natural substance consist in this that objects made from the artificial product possess greater strength and durability, and are easier to make and cheaper, than similar objects made from real meerschaum. It may be mentioned that real meerschaum and also the mass which is commonly used in pipe-manufacturing and which is made from the waste of real meerschaum becomes gradually soft or mellow in the course of time 40 through the influence of the air, so that their resistance to external influences diminishes more and more and they become less fit for service.

45 The artificial meerschaum produced according to this invention is however absolutely insensitive to the above mentioned influences of the time, of the air, of the smoke and the like so that the durability of the objects made according to the new process is 50 much greater than the durability of similar ornamental or useful objects made from real

meerschaum or from a mass produced from waste of real meerschaum.

The process according to this invention 55 consists in intimately mixing—preferably in a ball mill—Hallic earth and Meissner clay, or Meissner clay alone which in this case has to be partly in raw pulverized state and partly in roasted state, with whiting and 60 quartz dust, after the several substances have been finely pulverized and in adding water until all the granular substances have been ground, so that a semi fluid paste is formed, which is filtered if desired, through filter 65 paper, whereupon the paste or residue left on the filter (the filtrate being discarded) is slowly poured into moulds of gypsum and left to stand in these moulds for some time (several minutes will generally be sufficient), 70 so that a layer of the mass settles upon the inner surface of the mould. The remaining mass which has become thinly liquid (so called slip) is poured out of the mould and the moulded article is carefully removed 75 from the mould after it has sufficiently dried, whereupon the moulded article is baked in the oven at a temperature of about 800° C., oiled and waxed, mounted in bamboo or in 80 osier and lacquered.

It is necessary to let the moulded article dry in the mould as the mass which has settled in the required thickness upon the wall of the mould is still very soft and sensitive 85 after the remainder of the liquid has been poured off so that it could be easily damaged when taken out of the mould at once.

Hallic earth consists of:—  
56.68 SiO<sub>2</sub>, 30.63 Al<sub>2</sub>O<sub>3</sub>, 1.09 Fe<sub>2</sub>O<sub>3</sub>, 0.16 CaO, 0.31 MgO, 0.59 KNaO, 10.82 H<sub>2</sub>O, and 90 is obtained in the neighbourhood of Halle, on the Saale. The melting point of Hallic earth is about 32–34 Seger cone. Hallic earth is a form of kaolin while Meissner clay consists of:—

59.10 SiO<sub>2</sub>, 27.34 Al<sub>2</sub>O<sub>3</sub>, 0.76 Fe<sub>2</sub>, 0.10 CaO, 0.22 MgO, 0.43 KNaO, 11.85 H<sub>2</sub>O, and is obtained in the neighbourhood of Meissen, in Saxony. The melting point of Meissner clay is about 31–32 Seger cone. Meissner clay is a form of kaolin.

A mixture of the following composition is to be recommended:—

30 parts by weight of Hallic earth, 10

parts by weight of Meissner clay, 4 parts by weight of whiting, 8 parts by weight of quartz dust to which mixture when it is being treated according to the invention 50 parts by weight of water have to be added.

Articles of even better quality will be produced by the following mixture:—

34 parts by weight of Meissner clay, pulverized at the raw state,

10 14 parts by weight of Meissner clay, well roasted, pulverized,

6 parts by weight of quartz dust, washed, 7.5 parts by weight of whiting,

15 0.8 parts by weight of feldspar, 50 parts by weight of water.

The articles produced from the special means must be capable to be worked subsequently the biscuit baking, and the material must be of such a nature that it can be cut or scratched with the knife. Although the material, as regards composition has a strong resemblance to earthenware and more specially to limestone-ware it differs, owing to the special manner of baking, from earthen-ware or limestone-ware by the capacity to be cut or scratched with the knife, as earthenware or limestone-ware is hard and clinkering and cannot be cut with the knife. The special manner of baking mentioned above consists merely in maintaining a comparatively low temperature at the baking. While earthenware is submitted to a temperature from 1100 to 1300° C. the material is in this case only baked at a temperature of 800 to 1000°.

In order to produce a considerable reduction of the weight of the finished product and in order to ensure certain advantages in manufacturing e. g. in so far as the manufacturing of pipe-bowls and the like is carried out more rapidly than with the composition of the mass as stated above, and with a view to increase still further the resisting capacity against stroke and shock 40 and consequently the durability, infusorial silica is either substituted for the washed quartz or it is used as special addition. In the latter case the quantity of infusorial silica added can vary according to the required reduction of weight of the finished product, resulting from this addition.

To one kilogram of the mixture composed as stated above 200, 300, 400 and even up to 55 700 grams of infusorial silica can be added.

Magnesia could further be added in order to increase the flexibility of the mass, or carbonate of potassium which is generally used for this purpose.

The articles to be produced are obtained directly in the desired shape so that it is not necessary to bore out the mass as must be done in the manufacture of articles of real meerschaum, the cost of manufacture being thus reduced considerably so that the

articles made from artificial meerschaum according to this improved process are much cheaper than those made from real meerschaum or from the well known meerschaum mass.

The casting process itself is not new and is known in the manufacture of artificial masses which contain waste of meerschaum and show a certain likeness with meerschaum. I am aware that masses are known which are adapted to be cast and which contain clay, chalk, quartz and feldspar.

I claim:—

1. Process for the manufacture of artificial meerschaum consisting in finely grinding a substance commonly used for the manufacture of earthenware, composed of Hallic earth and Meissner clay with whiting and quartz dust, in adding water to said mass, in filtering the same to form a paste, in bringing the paste into well dried moulds, in letting the mass dry in the moulds, in removing the dry mass from the moulds and in giving the same the biscuit baking known in the manufacture of porcelain.

2. Process for the manufacture of artificial meerschaum consisting in finely grinding a substance commonly used for the manufacture of earthenware, composed of 90 30 parts by weight of Hallic earth and 10 parts by weight of Meissner clay, in admixing this substance with 10 parts by weight of finely ground whiting and with 4 parts by weight of finely ground quartz dust, in adding 50 parts by weight of water, in filtering the mixture to form a paste, in bringing 100 the filtered mass into well dried moulds to let the same dry, in removing the dried mass from the moulds and in submitting the same to the biscuit baking known in manufacturing porcelain.

3. Process for the manufacture of artificial meerschaum consisting in finely grinding a substance commonly used for the manufacture of earthenware, composed of 110 Hallic earth and Meissner clay with whiting and quartz dust, in adding water to said mass, in filtering the same to form a paste, in adding infusorial silica to the mass and in adding magnesia and carbonate of potassium to the mass in order to increase the 115 malleability of the same, in bringing the paste into well dried moulds, in letting the mass dry in the moulds, in removing the dry mass from the moulds and in giving the same the biscuit baking known in the manufacture of porcelain.

In testimony whereof I affix my signature in presence of two witnesses.

PAUL DEUSSING.

Witnesses:

BERNHARD R. REISER,  
SIGMUND LÖWENSTEIN.